

W. M. PAGE,  
PROCESS OF MAKING CLAD METALS,  
APPLICATION FILED JUNE 28, 1910. RENEWED JUNE 10, 1913.  
**1,084,474.** Patented Jan. 13, 1914.



Witnesses  
J. M. Offutt,  
D. T. Phelps.

Inventor  
W. M. Page  
by  
K. P. McElroy  
Attorney

# UNITED STATES PATENT OFFICE.

WILLIAM MARSHALL PAGE, OF PHILADELPHIA, PENNSYLVANIA.

## PROCESS OF MAKING CLAD METALS.

1,084,474.

Specification of Letters Patent.

Patented Jan. 13, 1914.

Application filed June 28, 1910, Serial No. 569,302. Renewed June 10, 1913. Serial No. 772,879.

*To all whom it may concern:*

Be it known that I, WILLIAM MARSHALL PAGE, a citizen of the United States, residing at Philadelphia, in the county of Philadelphia and State of Pennsylvania, have invented certain new and useful Improvements in Processes of Making Clad Metals, of which the following is a specification.

This invention relates to processes of making clad metals; and it comprises a method of making clad metals, and particularly copper clad steel, wherein a billet of metal is first film-coated to secure a weld united coating and is thereafter coated with a substantial body of metal by casting a body of coating metal through a restricted orifice into contact with such filmed surface; all as more fully hereinafter set forth and as claimed.

20 It is not easy to obtain a good, substantial and permanent union between steel and copper but such a union is now practicable by the processes of Patent #853,716 and by the methods of my copending application Serial 25 No. 467,651. If a clean steel surface be brought into contact with copper heated several hundred degrees above its melting point, a union can be effected, which on cooling will withstand violent temperature 30 changes and torsion to rupture, and which cannot be discovered by cleaving tools such as a cold chisel. Or if the steel surface be decarbonized so as to give a substantially carbon-free surface layer of iron, the union 35 may be effected by casting copper thereagainst at a lower temperature. This decarbonization may be effected by forming a coating of magnetic oxid on a steel billet, as by exposure to superheated streaming steam 40 and thereafter causing the magnetic oxid and the carbon of the underlying metal to react with each other to form pure iron, such iron coming both from the oxid and from the underlying metal. This reaction may 45 be performed by simply submerging the oxidized billet in molten copper. In the ordinary practice of making copper clad steel, it is customary to film coat the billet by dipping it into molten copper under the proper 50 conditions to secure a weld union and thereafter unite with the filmed surface a substantial body of the coating metal. This double coating operation is performed for several reasons. For one thing, it is a relatively expensive operation to maintain a 55 large body of coating metal in a highly

heated and carefully controlled state, and it is simpler and easier to use this body merely for film coating, putting on the main body of copper from another source. Furthermore, the copper which is used for dipping or film coating the billet is more or less contaminated by dissolved iron; and while for the purpose of producing the preliminary or film coating the presence of this iron 60 is desirable since it causes a readier union yet for electrical purposes it is highly desirable that the main body of the coating shall contain no iron or substantially none, 65 the presence of a fraction of a per cent. of iron in copper running down its conductivity inordinately. The double operation is therefore also desirable as permitting the main body of the coating to be made of specially purified metal.

In attaching the second and substantial coating of copper to the film coated billet many precautions are necessary. The molten copper must not be brought into contact therewith in such a way as to wash off the 70 film coating, since this would result in the diffusion of iron through the body of the copper. For the same reason of preventing contamination it is desirable not to use the molten copper for the substantial coating in 75 a highly heated state. The film coating being largely alloyed with iron is relatively fusible and is readily melted off.

In the ordinary practice of the double coating operation, the cleaned or oxidized 80 steel billet is placed in an open bottomed casing. This casing during the operation is maintained full of producer gas to obviate oxidation of the steel or of the copper coating. Billet and casing are hoisted together above a bath of copper of the proper 85 composition and temperature, the billet thrust beneath the surface of the molten copper and there maintained for a period of time sufficient to produce an alloying and 90 union of the two metals. The billet is now withdrawn from the copper into the casing, and as withdrawn it is found to be 95 covered with a thin clinging film of copper and copper iron alloy. The bottom of the 100 casing containing the filmed billet is next closed. This may be done by screwing a cap on the end of the filmed billet, the cap being one which is adapted to make a fluid-tight contact with the bottom of the casing, 105 The casing is provided with orifices near its top covered by a temporary seal of asbestos

cloth or the like. Casing, billet and cap are next lowered into another bath of copper of the desired purity, the casing being lowered until the copper covers and flows in through the orifices, the asbestos being removed. These orifices being of restricted size it is possible to keep them covered by a body of molten copper so that air cannot enter. The temperature of the copper and of the casing are preferably so correlated that the copper flowing in through the orifices shall solidify first next the wall while later entering copper progressively fills up the space between the copper already solidified and the filmed surface of the billet. The portion of copper which solidifies next the wall cannot become contaminated by iron from the film coating. The entering copper may run down and solidify next the wall 20 and be solidified as successive inward layers. Or it may enter in such a manner as to form, so to speak, a constantly upwardly growing rim of solidified copper next the mold wall with later solidifying liquid copper between this rim and the film coating. The important thing is to prevent contamination of the outer layers of copper, restricting all contamination by the film coating to the layers next thereto, this contamination being 30 rendered as slight as may be.

The dipping of the whole mold with an included billet in a bath of copper is an expensive and inconvenient operation. It requires a bath of copper of a size larger and depth greater than those of the casing, and practically only round casings can be used. But where it is desired to secure a high purity of the coating, as is the case with all clad metal intended for electrical purposes, it has not heretofore proved practicable to pour or cast melted copper directly into the mold at its top in the ordinary way of making castings. Direct casting does not give as good results for this purpose as this 40 operation of submerging mold, billet and all beneath the surface of a large body of molten copper. In direct pouring it is difficult to make the copper solidify next the mold wall prior to contact of the molten copper with the film without contamination from the filmed surface. And in pouring in, the molten copper passes into and through a body of air which it carries along with it into the mold, tending to make a blowy 50 casting and to become oxidized. The oxidation renders difficult a good union between the cast-in copper and the copper of the film. If the cast-in copper be hot enough to give a good gravitational separation of oxid it will wash or dissolve off the film coating and become contaminated.

In the present invention I have devised a new way of bringing the copper for the substantial coating into the mold which avoids the stated disadvantages of casting and ob-

tains the advantages of the dip-molding operation. In lieu of casting the copper directly into the space between the filmed billet and the mold body, I provide the mold body with one or more gutters or troughs 70 near its top communicating with the interior of the mold in the side wall through relatively small orifices. This gutter may or may not entirely surround the mold, this depending on the shape and size of said mold. The mold may be round or square or any other shape. With a round mold an annular gutter is convenient. Upon casting the copper into this gutter the conditions of the dip molding operation are simulated, a 75 body of copper covering and entering the restricted orifices in the side walls. During the entire casting operation, these orifices are kept covered and sealed by molten copper. The entering copper is caused to 80 solidify first next the mold wall as described. During the operation the mold may be kept full of producer gas. Under these conditions, oxidation is obviously impossible. Whatever oxid is formed in casting through 85 the air remains with the copper in the trough. Enough copper should be cast into the trough to keep the orifices covered while the main body of the coating is formed. By ceasing to pour at this time, this sealing 90 copper (which will be contaminated by gas and floating oxid) runs in above the top of the billet whence it can be later removed. Or by providing the casing with minute orifices above the level of the end of the intended coating on the billet, this last copper 95 can be again drained out. By casting copper into the gutter and maintaining enough copper there to cover the orifices during the casting operation proper, no air can be 100 passed into the mold. As stated, at the completion of the casting, the excess of copper 105 may be drained out through these small orifices in the side of the mold, which may be provided with a suitable closure.

The coating operation is made much more flexible by the described process since the size and shape of the mold need not conform to the dimensions and shape of the vessel containing the molten copper as is necessary 115 in dip-molding. The mold can be square or of any shape desired, and need not be the protective casing employed during the film coating operation but may be a separate piece of apparatus. One filming casing may 120 supply filmed billets for a number of heavy coating molds. And since there is no need of submerging a strong and heavy mold in the molten copper at any stage of the operation cheaper casings and molds may be employed.

In the accompanying illustration I have shown, more or less diagrammatically, means and material for accomplishing the described process. In this showing the 130

figure represents a vertical section of the apparatus.

Element 1 is a furnace chamber shown as lined with refractory material 2. This chamber as shown is of generally cylindrical shape and is intended to be fired by oil flames or the like, from end burners, (not shown). The furnace chamber is mounted for tilting upon rollers 3, and is provided with counterpoise means 4. The furnace chamber is further provided with a port 5 which may be closed by swinging door 6. Through this port it may be replenished with metal and the port also serves as a waste gas removing means. It is also provided with a side duct 7 leading to an offset pocket 8. This pocket is provided with a dipping port 9, which may be merely large enough to admit a billet, or may admit also the end of the filming casing, and with a pouring lip 10. Ram 11 allows the tilting of the furnace into any desired position. When swung into one position the copper will flow back into the flame chamber while when swung into another the molten copper will, as shown, accumulate in the dipping pocket. This enables the copper to be purified, heated and treated in one chamber and then transferred to another for filming without danger of intermediate contamination. The mold or casing 12 is shown as adapted for both filming and coating and as containing a billet 13, carried by porterbar 14. This porterbar and the hoisting means 15 allow independent motion of casing and billet. Near the top of the casing are inlet orifices 16 which may be covered and sealed by a strip of asbestos or the like 17. Connecting with these orifices is a gutter or channel 18 which may or may not be continuous around the mold, this depending on convenience. As shown, the mold or casing is round and provided with a continuous annular gutter. A neutral atmosphere may be maintained in the casing during the various operations by means of gas, such as producer gas, passed in through 19. At its base, the billet may carry a cap 20 adapted to seat and engage with ribs 21 of the casing to make a fluid-tight joint. The cap may be screwed to the billet by screw threaded means 22 (shown as exaggerated in size). In the molding operation proper, copper may be cast into the gutter either from the pouring lip of the coating furnace described, or from a separate crucible or ladle 23. The mold is provided with small venting or draining orifices 25 which may be kept closed by band 26.

In the use of the described apparatus the coating furnace may be tilted into a position where the copper will flow back into or remain in the cylindrical chamber shown. Here it may be heated and brought to any temperature desired, and may also be puri-

fied. During this operation door 6 will be closed, and the flame gases will escape through dipping port 9, which now serves as a waste gas exit. This serves to heat the dipping pocket. When the copper is 70 brought to the proper temperature and composition the furnace is swung into the position shown in the drawing, when the copper will flow into the dipping pocket, the waste gases now escaping through 5, door 6 75 being swung out of the way for this purpose. The casing is lowered to or into the dipping port and the billet 13, which has been previously treated in any way desired, is lowered into the molten copper and main- 80 tained beneath its surface until the desired amount of alloying has taken place and it is provided with a weld-united film. It is now raised and brought back into the casing, cap 20 affixed, if not already attached, and 85 caused to make a tight joint with the bottom of the casing. The billet and casing are now placed upon floor 24, the asbestos seal 17 removed and copper poured into the casting channel, this copper coming from 90 pouring lip 10 or from ladle 23, and being of any special composition and temperature desired. Or, alternatively, in lieu of attaching the end cap to the billet and using the protective casing as a mold, the filmed 95 billet may be removed from the first dip coating casing and lowered into another mold for the coating operation. For electrical goods, the coating copper is best taken from another furnace than the one which is 100 serving for the dipping operation since, as stated, in the dipping the copper is contaminated more or less by iron. The contamination by iron of the copper in the furnace shown after the filming operation may how- 105 ever be obviated and certain advantages gained by then tilting the furnace back into the melting position and burning out the dissolved iron from the copper. When iron is dissolved in copper, as it is in the filming 110 operation, it effectually removes dissolved oxids and oxygen, while the excess of iron may be effectually removed by a subsequent preferential oxidation without re-oxidizing the copper. In this preferential oxidizing 115 operation the surface of the molten copper should be covered and protected by floating carbon, such as charcoal or coke, and flame then impinged on the protected surface. Under these conditions, iron will burn out, 120 leaving the copper pure and unoxidized. In the presence of the carbon, the surface of the steel is blanketed by carbon dioxid and carbon monoxid gases, both of which have an oxidizing effect on iron but not on copper. 125 The purified copper may now be employed for the main coating by casting into the gutters of the mold. In practice, the copper in a given furnace may be employed for dipping a number of billets, thereby becoming 130

purified from oxygen and oxids and contaminated by iron, may then be treated to remove the dissolved iron and then be used for billets filmed in another similar furnace.

5 But in the ordinary course of the work it is generally better to use a separate supply of copper for the main body of coating. This may be melted and purified in crucible 23 which then may be used as a ladle. Two 10 such furnaces as those shown may be used in alternation, one being used for the dipping operation until the copper is free of oxygen but full of dissolved iron, while the other is supplying purified, copper, and conversely.

15 In making electrical materials, the mold used for the coating operation is preferably kept during the coating operation at such a temperature that the inflowing copper will solidify next its walls in the manner described.

In the casting operation, the copper accumulates in the gutter above the level of the restricted orifices, sealing them against entrance of air or entangled oxid. The oxid 25 formed in pouring through the air, remains floating on the pool of copper while clean copper is tapped into the mold through the orifice below the copper surface. This sealing by molten copper is maintained throughout the time needed to introduce enough copper to fill the space between the mold walls and the filmed billet. After the copper rises above the end of the billet, entrance of air and oxid is unimportant. In other words, 30 the copper is cast into the gutter at a somewhat greater rate than it can pass therefrom into the mold through the restricted orifices. At the end of the pouring, the molten copper in the gutter passes into the mold where it may remain to solidify and later be cut off; or it may be again drained away through drain holes 25, sealing band 26 being removed. During the casting operation, 35 the head of molten copper in the gutter should not be high enough to cause any very forcible projection inward into the mold or any spouting inward flow.

What I claim is:—

1. The process of making clad metals which comprises placing a billet of core metal within a suitable mold casing and casting molten coating metal into a channel communicating with the interior of said mold through a restricted orifice in its side until a coating is formed, the size of the orifice and the speed of pouring being so correlated that liquid coating metal remains in said channel above the level of and seals said orifice until the coating is formed.
2. The process of making clad metals which comprises placing a billet of core metal within a suitable mold casing and casting molten coating metal into a channel communicating with the interior of said mold through a restricted orifice until a

coating is formed, the size of the orifice and the speed of pouring being so correlated that liquid coating metal remains in said channel above the level of said orifice until the coating is formed, and the temperature of said mold and of said molten metal being so correlated that entering metal first solidifies next the inner wall of the mold while later solidifying metal fills up the space between said first solidified metal and said billet.

3. The process of making clad metals which comprises placing a billet of steel within a suitable mold casing and casting molten copper into a channel communicating with the interior of said mold through a restricted orifice in its side until a coating is formed, the size of the orifice and the speed of pouring being so correlated that liquid copper remains in said channel above the level of said orifice until the coating is formed.

4. The process of making clad metals which comprises placing a billet of steel within a suitable mold casing and casting molten copper into a channel communicating with the interior of said mold through a restricted orifice until a coating is formed, the size of the orifice and the speed of pouring being so correlated that liquid copper remains in said channel above the level of said orifice until the coating is formed, and the temperature of said mold and of said molten metal being so correlated that entering metal first solidifies next the inner wall while later solidifying metal fills up the space between said first solidified metal and said billet.

5. The process of making copper clad steel which comprises film-coating a steel billet with copper, maintaining the filmed billet within a suitable mold casing and casting molten copper into a channel communicating with the interior of said mold through a restricted orifice until a coating is formed, the size of the orifice and the speed of pouring being so correlated that liquid copper remains in said channel above the level of said orifice until the coating is formed.

6. The process of making copper clad steel which comprises film-coating a steel billet with copper, maintaining the filmed billet within a suitable mold casing and casting molten copper into a channel communicating with the interior of said mold through a restricted orifice until a coating is formed, the size of the orifice and the speed of pouring being so correlated that liquid copper remains in said channel above the level of said orifice until the coating is formed, and the temperature of said mold and of said molten metal being so correlated that the entering metal first solidifies next the inner wall while later solidifying metal

fills up the space between said first solidified metal and said billet.

7. The process of making copper clad steel which comprises maintaining a copper-filmed steel billet within a suitable mold casing carrying an exterior channel communicating with the interior of said casing through a restricted orifice and casting molten copper into said channel in such manner that fluid copper remains in said channel above said orifice until sufficient copper has entered the casing to fill up the space between the billet and the casing.

8. The process of making copper-clad steel which comprises film-coating a steel

billet with copper, maintaining the filmed billet within a casing containing an indifferent atmosphere and casting molten copper into a channel communicating with the interior of said casing through a restricted orifice, the level of the molten copper in said channel being maintained above said orifice until entering copper has filled the space between said billet and the mold casing.

In testimony whereof, I affix my signature in the presence of witnesses.

WILLIAM MARSHALL PAGE

Witnesses:

P. M. WEIS,  
JOHN B. PATTON.